

## UNITED STATES PATENT OFFICE

1,930,463

## HARDENING OF ALUMINUM

Robert S. Archer, Milwaukee, Wis., assignor to  
 Aluminum Company of America, Pittsburgh,  
 Pa., a corporation of Pennsylvania

No Drawing. Application March 4, 1931  
 Serial No. 520,155

5 Claims. (Cl. 148—7)

The invention, which relates to aluminum and aluminum base alloys, is directed to a process for producing aluminum or aluminum alloy products having a surface of a hardness substantially greater than the hardness of the interior metal.

For purposes of simplicity, the word "aluminum" as used herein and in the appended claims is defined to include not only pure metallic aluminum but also aluminum in all commercial grades 10 of purity as well as aluminum base alloys containing more than about 50 per cent of aluminum.

Among the commercial metals and alloys, aluminum is relatively soft and ductile. Alloys of aluminum have been produced and heat-treatments suited to these alloys have been devised, resulting in the development of alloys of relatively high mechanical properties. However, whether an increase in hardness has been obtained by alloying methods, by cold working the metal, or by 15 thermal treatments, the ductility of the aluminum decreases to some extent as the hardness increases and aluminum treated by these methods of hardening may become quite brittle. In many instances where hardness is the desideratum, it is 20 only surface hardness that is required and it becomes immaterial if the hardness of the interior of the metal does not equal that of the surface. In fact, it is as often advantageous that the metal present a hard exterior surrounding a more yielding and ductile interior. Such soft core articles are characterized by high surface resistance to 25 wear, yet withstand the sudden shocks or repeated stresses encountered in service. For instance, at the present time, a large number of pistons for 30 internal combustion engines are made of aluminum, the number annually sold amounting into the millions, but there is, nevertheless, a widespread demand for a more wear-resistant aluminum piston which will retain all the desired characteristics of the aluminum now used but which 35 will present a harder and, consequently, more wear-resistant surface.

Because of the demand for such articles, I have been led to devise my present invention 40 which consists in packing the aluminum article to be treated in a mass of comminuted magnesium metal in such manner and under such conditions that the surface of the article and the particles of the magnesium powder are in close and 45 intimate contact, and thereafter subjecting the thus packed aluminum article and comminuted magnesium metal to a thermal treatment for such lengths of time and at such temperatures as will produce the results hereinafter described.

50 Preliminary to packing the aluminum article

in the magnesium metal, the surface of the article is preferably treated so that it will be substantially free from dirt, oil, oxides, or other extraneous material. I have found that exceptionally good results are obtained if the cleaning operation employed is one which roughens the surface of the article slightly. To accomplish such a surface cleaning, the aluminum article may be rubbed with an abrasive or treated with a solution of an acid or alkali, or a combined treatment 60 may be used. These are usual methods of cleaning aluminum surfaces and similar and other well known methods may likewise be used with satisfactory results. The comminuted magnesium metal in which the aluminum article is then packed should preferably be of a pure grade and in a comparatively fine state of subdivision. One form of comminuted magnesium metal which I have found effective is sometimes known as "cutter material" and consists of the fine chips and 65 curls of metallic magnesium produced by machining a magnesium ingot. Magnesium powder as it is sold in commercial form and other similar forms of comminuted magnesium metal are also satisfactory.

The aluminum article may be packed in the comminuted magnesium metal in any suitable receptacle which fits conveniently in the heating furnace which is to be employed. Because, however, of the propensity of magnesium metal to 70 oxidize readily and even ignite at high temperatures, I have found it necessary to exclude during the heating process any substantial quantity of air. It is possible to obtain satisfactory results by placing the comminuted magnesium metal and 75 the aluminum article packed therein in an airtight receptacle but I prefer to accomplish this purpose during heating by introducing into the heating furnace an atmosphere of some gas which is inert to magnesium, such as carbon dioxide, 80 which will preclude the necessity of the use of airtight receptacles.

The aluminum article packed in the comminuted magnesium metal is then, in accordance with my invention, heated to a temperature sufficient to cause diffusion of the magnesium into the surface of the aluminum article. The temperature at which such diffusion becomes rapid enough to be commercially practicable is usually 85 above about 250° centigrade when a close and 90 intimate contact between the magnesium metal and the surface of the aluminum article exists. For rapid diffusion, however, I find it preferable 95 to heat the packed article at temperatures in the neighborhood of about 420° centigrade to about 100 105 110

460° centigrade, but since the eutectic mixture formed by the aluminum and magnesium or by the diffusion of the magnesium into the aluminum melts at about 450° centigrade, it is not desirable to substantially exceed that temperature although a small amount of incipient fusion upon the surface of the aluminum article will not be deleterious in effect. If, however, there is a possibility of incipient fusion at the points of contact between the comminuted magnesium metal and the aluminum article and such incipient fusion is not desired, I have found it to be beneficial to add about 5 per cent by weight of magnesium oxide to the comminuted magnesium metal since it appears that the added magnesium oxide acts as a diluent and produces a more uniform surface hardness.

The time for which the heating should be carried out depends upon the temperature, a higher temperature requiring a shorter time to produce a given result. The effect of my novel treatment is to produce on the aluminum article a hardened surface, which surface is composed of an alloy of aluminum and magnesium, and the depth of which depends upon and increases with the temperature employed and the time of treatment. The existence, extent, and depth of the hardened surface may be readily determined by microscopic examination or by testing the surface with a file. Aluminum articles treated in accordance with my invention can be machined, filed, or cut more easily than untreated articles, and are also capable of taking a high polish.

The article produced in accordance with my invention is characterized by the fact that the surface formed on the aluminum article is not readily distinguishable chemically, mechanically, or visually from the metal of the core. The surface is not magnesium per se but is an alloy of aluminum and magnesium formed by the diffusion of the magnesium into the outer surface of the treated aluminum article.

Exemplary of the practice of my invention is an instance where an aluminum base alloy containing 13 per cent of silicon was packed in comminuted magnesium metal and heated for 20 hours in an air-tight receptacle at a temperature of about 440° centigrade. The article after treatment had a surface hardness of 26 as measured by the scleroscope, while the interior metal or core had a hardness of only 9. An aluminum base alloy containing 4 per cent of copper and inherently harder than the aforementioned silicon alloy had, after a similar treatment, a surface

55

hardness of 29 and a core hardness of 21. Thermal treatments subsequently applied to articles which have been treated in accordance with my invention for the purpose of modifying or producing certain properties of the aluminum may change the actual hardness of both the surface and interior of the metal but a relative hardness differential produced as the result of my novel treatment will usually be retained.

Having thus described and explained my invention and the method in which it may be practiced, I claim:

1. A method of increasing the hardness of an aluminum article at or near the surface, comprising packing the aluminum article in close and intimate contact with comminuted magnesium metal and heating the packed article at temperatures above about 250° centigrade and below about 460° centigrade. 90

2. A method of increasing the hardness of an aluminum article at or near the surface, comprising placing the aluminum article in close and intimate contact with a comminuted material comprising magnesium, and heating the article and comminuted material to a temperature above about 250° centigrade and below about 460° centigrade while excluding substantial amounts of air therefrom. 95

3. An aluminum alloy article having a relatively soft interior core and a relatively hard exterior surface, the said exterior surface consisting of an alloy of aluminum and magnesium formed by diffusion. 105

4. A method of increasing the hardness of an aluminum article at or near the surface, comprising placing the aluminum article in close and intimate contact with comminuted material comprising magnesium metal and magnesium oxide and heating the article and comminuted material to a temperature above about 250° centigrade and below about 460° centigrade. 110

5. A method of increasing the hardness of an aluminum article at or near the surface, comprising placing the aluminum article in close and intimate contact with a comminuted material comprising magnesium, and heating the article and comminuted material to a temperature above about 250° centigrade and below about 460° centigrade while substantially excluding air therefrom until magnesium diffuses into said article and alloys therewith and increases the surface hardness thereof, substantially as described. 115

ROBERT S. ARCHER.

130

60

135

65

140

70

145

75

150